

# UNITED STATES PATENT OFFICE.

MURTY CUNNINGHAM, OF BELLEFONTE, PENNSYLVANIA.

## COMPOSITE PAVEMENT.

SPECIFICATION forming part of Letters Patent No. 398,946, dated March 5, 1889.

Application filed September 3, 1888. Serial No. 284,442. (No specimens.)

*To all whom it may concern:*

Be it known that I, MURTY CUNNINGHAM, of Bellefonte, in the county of Centre and State of Pennsylvania, have invented a new and Improved Composite Pavement, of which the following is a full, clear, and exact description.

This invention relates to artificial pavements, and has for its object to provide a pavement which will be effective and durable.

The invention consists in a composite pavement constructed and arranged as hereinafter described; in a composition for such pavements, consisting of broken stone or its equivalents, coke-screenings or screened coal-ashes, coal-tar, sulphur, a coloring material, and tallow, mixed for use, as hereinafter set forth.

The invention further consists in the application to the top layer of the pavement of a mixture of coal-tar, sulphur, a coloring material, and tallow while hot, all as hereinafter more specifically set forth and claimed.

My composition comprises, first, a body mixture consisting of four bushels coke-screenings or screened coal-ashes and two bushels of ore-flint, gravel, broken stone, or broken iron cinders of a size of from one and one-fourth to one and three-fourths inch, well incorporated together, and of a binding mixture of six gallons of coal-tar, one pound sulphur, one-half pound tallow, and one-quarter pound Prussian blue. This second mixture is to be heated so as to be thin enough to mix well with the first mixture. After the two mixtures have been thoroughly incorporated together the composition can be put aside in a pile and another batch made up in the same proportions until the required quantity is prepared. If made up weeks beforehand, it will be better for use, as its paving qualities are not developed until put in place and rolled thoroughly.

One or more layers of the composition will be required, according to the depth of pavement called for. For street-pavements where heavy wagons are used it should be about five inches thick.

In putting down my improved pavement I first provide a suitable foundation of any suitable material—as broken stone, gravel, cinders, coal-ashes, &c.—which is rolled even and

solid, so that the pavement when finished will be uniform in thickness; but any foundation will answer. I then put over the foundation a layer of the composition about one and a half to two inches in thickness, and roll it so as to form a solid mass. As many layers are thus put down as will make within about three-quarters of an inch of the required thickness of the pavement. I then put on a layer of the same mixture, but with the stone or its equivalent broken to a size of from one and a quarter to one and three-quarters of an inch, which is then rolled solid and smooth. I then take a quantity of mixture No. 2, heated until very thin, pour it over the surface, and scrub it with a broom, so as to fill all crevices and harden the surface. The surface is then covered with sharp sand, so that the tar will not be seen. The pavement is then ready for pedestrians, and the more sand is tramped in the smoother the pavement.

This composition will adhere whether laid on clay, stone, iron, or brick, and can be used for any pavement for cross-walks or for lawn-walks.

The great objection heretofore to this class of pavement has been the length of time required for it to harden; but the addition of the sulphur entirely obviates this objection, as the sulphur causes the composition to harden quickly.

The tallow and Prussian blue make a lasting color which does not fade, the pavement retaining a bright blue color.

It will be understood that the tallow and Prussian blue might be omitted from the second mixture when used in the composition for the lower layers in a pavement, as its purpose is mainly to give color to the pavement. It is also to be understood that the materials for the first mixture may be varied according to the location and ease of obtaining the same. Coke-screenings are preferred as making the best paste, but ashes answer when the coke cannot be had; also, the iron ore flint, which can be obtained anywhere where iron ore is raised and can be obtained of the proper size, makes the best material for the purpose; but either of the other articles named or any similar material will answer the purpose; and it will be further understood that although broken stone

and screenings are specifically claimed any equivalent thereof may be used without departing from the spirit of my invention.

Having thus described my invention, what I claim as new, and desire to secure by Letters Patent, is—

1. In compositions for pavements, a binding mixture consisting of coal-tar, sulphur, tallow, and a coloring material, combined substantially in the proportions set forth.
2. A composition for pavements, consisting

of broken stone, screenings, coal-tar, sulphur, tallow, and a coloring material, combined substantially in the proportions set forth.

3. A composition for pavements, consisting of broken stone, coke-screenings, coal-tar, sulphur, tallow, and Prussian blue, substantially as described.

MURTY CUNNINGHAM.

Witnesses:

W. K. LUDWIG,  
W. J. HOWLEY.